

## UNITED STATES PATENT OFFICE.

DANIEL SNYDER GUSTIN, OF EAST ORANGE, NEW JERSEY, ASSIGNOR TO WESTINGHOUSE LAMP COMPANY, A CORPORATION OF PENNSYLVANIA.

GAS-FILLED INCANDESCENT ELECTRIC LAMP WITH FILAMENT HAVING INCREASED STRENGTH.

No Drawing. Application filed November 29, 1924. Serial No. 752,942.

This application is a continuation-in-part of my copending application, Serial No. 639,460, filed May 16, 1923, gas-filled incandescent lamps and getters therefor and assigned to the Westinghouse Lamp Company.

This invention relates to incandescent electric lamps and more particularly to gas-filled lamps in which a metal filament there-in is given an increased strength by the use of a getter, such as diphenyl amine or an equivalent organic compound.

An object of my invention is the use of a getter especially adapted for gas-filled incandescent electric lamps and of such a character that an improvement in the strength of the metal filament and lumen maintenance during life, results.

Another object of my invention is the application of a getter in a gas-filled incandescent electric lamp of such a character, that the crystal structure of the metal filament is substantially improved.

A further object of my invention is the employment of a getter in a gas-filled incandescent electric lamp, which getter is adapted to efficiently remove moisture and thereby make it possible to employ a cold exhaust for such lamps or exhaust at any temperature.

A still further object of my invention is the manufacture of gas-filled electric lamps, into the bulbs of which is introduced diphenyl amine with the gas filling.

Other objects and advantages of the invention will become apparent as the description proceeds.

In my aforementioned copending application, of which the present application is a continuation-in-part, I have described getters which may be used, either applied to the filaments of lamps or introduced with the gas filling thereof, whereby the necessity for heating the bulbs thereof during exhaustion is obviated, because such materials are very efficient for removing moisture, as well as other materials, such as oxygen and nitrogen.

Although benzidine, or di-para-diamino-diphenyl,  $(\text{NH}_2)_2(\text{C}_6\text{H}_4)_2$ , has been found to be the preferred organic compound for introduction on the filament of the lamp, whereby cold exhaust may be utilized, yet I have found that when using diphenyl amine,  $\text{NH}(\text{C}_6\text{H}_5)_2$ , I effect, in addition, a

very desirable result, in that the strength of the filament is very materially increased, and the lumen maintenance during life is also improved.

I preferably introduce a vaporizable material such as diphenyl amine, which is a preferred example of an organic getter for increasing filament strength, with the gas filling for the lamp; yet, if desired, similar materials, having lower vapor pressures, might be applied directly to the filament, by means of a vehicle such as water or alcohol, in the form of a solution or suspension.

My invention will better be understood by the following more detailed description thereof.

I preferably place my getter, in solid form, in a tube and allow the filling gas to pass through the tube and over or thru the getter. The vapor tension of my preferred getter, diphenyl amine, is such, that a sufficient proportion is taken up by the inert filling gas, when substantially saturated therewith, to act on the metal filament to the desired extent. The bulb of the lamp is evacuated, either hot or cold and filled with said gas, either with or without preliminary flushing with nitrogen. The lamp is then tipped off and the filament flashed.

In order to show more clearly the improved results which may be secured by using diphenyl amine as a getter in metal filament, gas-filled, incandescent, electric lamps, the following results are tabulated below:

Average bump test results.

|                     | Number of test lots | Seasoned strength  | 90  |
|---------------------|---------------------|--------------------|-----|
| With getter.....    | 21                  | 80                 |     |
| Without getter..... | 3                   | 49                 | 95  |
|                     |                     | Overnight strength |     |
| With getter.....    | 9                   | 69                 |     |
| Without getter..... | 9                   | 35                 | 100 |

Average of life tests.

|                     | Burnout life | Standard spec. life | 105 |
|---------------------|--------------|---------------------|-----|
| With getter.....    | 1,382 Hrs.   | 2,648 Hrs.          |     |
| Without getter..... | 1,266 Hrs.   | 1,946 Hrs.          |     |

*Average per cent of initial lumens during life.*

|                | Per cent. |
|----------------|-----------|
| With getter    | 97.4      |
| Without getter | 93.8      |

5 The foregoing results clearly indicate that on bump test, the strength of the refractory metal or tungsten filament shows a material increase, both immediately after seasoning and after burning over night at 115% of 10 normal or rated voltage.

From the life test results, it will be seen that by using this getter, the burnout life is substantially lengthened as well as the standard specification life, which is a calculated 15 life, based on efficiency as well as actual life, and the average percent of initial lumens during life is materially increased.

Although, as aforementioned, it is preferred to introduce diphenyl amine, or its 20 equivalent, with the gas filling, yet equivalent materials or substitutes having lower vapor pressure, so that they would not evaporate from the filament during exhaust, might be applied directly upon the filament 25 by dipping, spraying or otherwise applying before mounting. For example, a weak solution, such as a 2% alcoholic solution may be used for this purpose. The mounted filament may be sealed into the lamp bulb 30 in the usual manner, the lamp exhausted either hot or cold, after which the desired gas filling may be introduced either with or without a preliminary flushing with nitrogen. The lamp may then be tipped off, the 35 filament flashed, and it will be found that not only does the strength of the filament increase, but the other desirable results aforementioned are obtained.

Although diphenyl amine has been mentioned 40 as the preferred material for a getter, according to my invention, I do not wish to be restricted thereto, as various other materials, of the same character, substantially free from oxygen or oxidizing material, may 45 be used. For example, it should be noted that ortho-amino-diphenyl,  $\text{NH}_2\text{C}_6\text{H}_4\text{C}_6\text{H}_5$ , an isomer of diphenyl amine, although not as desirable as diphenyl amine, may be employed, with good results.

50 The foregoing invention has proved so successful that it is now in commercial use on a large scale.

Although I have described what is now considered a preferred embodiment of my invention, it is to be understood that the 55 same is merely illustrative and that other modifications may be made within the spirit and scope of the appended claims.

What is claimed is:

1. An incandescent, metallic filament electric lamp of the gas-filled type, containing an organic material improving the resistance of the filament to shock. 60

2. An incandescent electric lamp of the gas-filled type, containing a getter composed 65 of diphenyl amine.

3. An incandescent electric lamp of the gas-filled type, containing a gas filling impregnated with diphenyl amine.

4. An incandescent electric lamp of the 70 gas-filled type, comprising a non-carbon filament surrounded by a gas filling impregnated with diphenyl amine.

5. An incandescent electric lamp of the gas-filled type, comprising a refractory 75 metal filament surrounded by an inert gas filling substantially saturated with diphenyl amine.

6. A getter suitable for improving resistance of metal filaments to shock when used 80 in gas-filled incandescent electric lamps, comprising an organic compound, substantially free from oxygen and oxidizing material.

7. A getter suitable for gas-filled incandescent electric lamps, for improving the 85 resistance of metal filaments to shock, comprising diphenyl amine.

8. The method of manufacturing incandescent electric lamps of the gas-filled type, 90 comprising sealing a filament into a bulb, exhausting the bulb cold and replacing the exhausted air by an inert gas containing diphenyl amine.

9. The method of increasing the strength 95 of refractory metal filaments in incandescent electric lamps of the gas-filled type, comprising introducing an inert gas filling substantially saturated with diphenyl amine.

In testimony whereof, I have hereunto 100 subscribed my name this 28th day of November 1924.

DANIEL SNYDER GUSTIN.